

Jan. 12, 1965

B. R. HARRIMAN

3,165,458

ELECTROLYTIC RECORDING SHEETS

Filed Sept. 22, 1961

FIG. 2



FIG. 1



FIG. 4



FIG. 3



INVENTOR  
BENJAMIN R. HARRIMAN

Carpenter, Abbott, Coulter & Kinney  
ATTORNEYS

1

3,165,458

## ELECTROLYTIC RECORDING SHEETS

Benjamin R. Harriman, St. Paul, Minn., assignor to Minnesota Mining and Manufacturing Company, St. Paul, Minn., a corporation of Delaware

Filed Sept. 22, 1961, Ser. No. 140,032

10 Claims. (Cl. 204—18)

This invention relates to new and useful sheets for the reproduction of visible images. In one aspect, this invention relates to improved image recording sheets which can be developed by electrolytic techniques. In another aspect, this invention relates to a method for the preparation of such sheets and to a method for their use in image reproduction.

Photoconductive coatings and sheet constructions have been suggested for a variety of purposes, including the reproduction of light images. A recently developed image reproduction process involves electrolytically developing permanent and visible images on suitable photoconductive copysheets after exposure to actinic light images. This method, described more fully in United States patent application, Serial Number 575,070, filed March 30, 1956, now U.S. 3,010,883, includes the electrolysis of an electrolytic developer and particularly the electrodeposition of a metallic or other visibly distinct coating at the exposed photosensitive surface, usually by electrolytic reduction. No preliminary charging of the copysheet is required, and the copy produced needs no further heating or other processing to render the image permanent. However, the successful application of the electrolytic method has been found to require, among other things, that the sensitive sheet be strongly photoconductive and have certain other conductivity requirements rather than merely the capacity to hold and dissipate an electrostatic charge. These copysheets, disclosed in greater detail in United States patent application, Serial Number 692,529, filed October 28, 1957, now U.S. 3,010,884, generally comprise a photoconductive layer of zinc oxide particles in an insulative organic resinous binder superimposed on a contiguous electrically conductive layer, the combined layers having a conductivity of at least about  $10^{-7}$  mho/cm. on exposure to 1300 foot candles of incident light from a tungsten source at 3100° K. (i.e. light conductivity) and a dark conductivity not greater than about one-twentieth of the light conductivity. Copysheets employing photoconductive indium oxide and their preparation are described in United States patent application Serial Number 848,219, filed October 23, 1959.

In attempting to improve the quality of such photoconductive copysheets, various means for increasing the image density and contrast, using electrolytically reducible developer materials, such as silver salts, have been investigated. Heretofore, the optical diffuse reflection density of a silver image has tended to reach a maximum of about one regardless of exposure or quantity of silver deposited in the image areas, and the average gradient of diffuse reflection density vs. log exposure curve, which is a measure of contrast, has been less than one. Such values are too low for printing average continuous tone photographic negatives. Furthermore, the density has been inadequate for many line copy and half-tone copy applications. Moreover, an increase in image density must be achieved without "pinpointing" (i.e. electrolytic breakdown of the photoconductive coating, causing points of heavy developer deposit), without yellowing or discoloration of the sheet, and without loss of the other desirable properties of such copysheets, e.g. good definition, ease and speed of development.

It is therefore an object of this invention to provide an improved photoconductive copysheet.

2

Another object of this invention is to provide a photoconductive copysheet which can be electrolytically developed to produce a visible image having improved image density, greater image contrast and better smudge resistance.

Still another object of this invention is to provide an improved photoconductive copysheet which is resistant to pinpointing and to yellowing.

A further object of this invention is to provide a photoconductive copysheet of improved appearance.

Yet another object of this invention is to provide a process for preparing an improved photoconductive copysheet.

Another object of this invention is to provide a means for preparing photoconductive copysheets having different degrees of gloss.

Other objects and advantages will become apparent from the following disclosure and examples.

An improved photoconductive copysheet of this invention comprises a continuous electrically conductive layer having thereon a thin, continuous and contiguous layer of photoconductive particles in a water-insoluble, insulative binder and, superimposed thereon, though not necessarily in direct contact therewith, a thin, continuous, glossy, adherent, transparent, cohesive, water permeable and water insoluble layer comprising a film forming silica. The silica must have film forming properties, as distinct from the silicas which dry from the aqueous sol to non-cohesive, readily disruptable powder. The former silicas are capable of forming a stable colloidal sol with a particle size in the 1 to 100 millimicron diameter range, preferably from about 10 to about 50 millimicrons.

Those silicas which are capable of producing the desired glossy, adherent, cohesive, water permeable layer are available as aqueous colloidal sols with up to about 50% solids in the above particle size range, which sols are of high purity and are substantially free of alkali metal cations, e.g. sodium, potassium, etc. They may be prepared by the progressive growth in aqueous sodium silicate solution of silica particles, such silica forming on nuclei of silicic acid. The alkaline sol thereby produced is deionized to remove sodium ion and reduce the pH to below 5, preferably below 4, by passage through an ion exchange bed. Such procedure is described in United States Patent No. 2,244,325. An illustrative silica sol is Nalcoag 1034A, a deionized acid sol containing 34% solids by weight and a particle size range of 16 to 22 millimicrons (available from Naco Chemical Company, Chicago, Illinois). Other Nalcoag silica sols, such as

those identified as 1015, 1022, 1030, 1035 and 1050, are suitable after deionization. Silica sols sold by E. I. du Pont de Nemours and Co., Wilmington, Delaware, under the trade name "Ludox" may also be used after deionization. Chemically modified silicas, e.g. esterified silicas, having the above properties may also be used. The pyrolytically produced silicas, though readily dispersible in water, are generally incapable of forming the desired glossy and continuous, cohesive film on the photoconductive copysheet surface. Additional ion exchange treatments of available film forming silica sols may be desired to remove traces of undesirable alkali metal cations, such as sodium ion, and hence to reduce the tendency of the top-coated photoconductive copysheet to pinpoint during electrolytic development. For example, less than 100 parts per million of sodium ion (calculated as NaOH) is preferred.

The various silica sols may be readily evaluated for suitability as film-forming silica sols and for other of the aforementioned properties by dip coating a ground, non-corrosive microscope slide into the silica sol, and removing and drying either with a hot air current or at ambient room conditions. The surfaces of the slide

should be previously ground with a fine abrasive, i.e. a grit size in the 320 to 500 mesh range. The useful silica sols will dry without blushing to a water insoluble film that reduces the dispersivity and increases the transparency of the ground glass surface. Aqueous solutions of dyes such as methylene blue will be strongly adsorbed on the coated surface and are not substantially removed by rinsing in water. If the silica sol provides too thick a coating, as evidenced by crazing or cracking of the film, the sol is diluted with water to reduce the coating thickness and the test is repeated. In distinct contrast to the useful silica sols, other silica sols of a non-film forming nature evidence blushing upon drying and will not dry to a coating having any significant transparency. Moreover, the non-film forming silica coatings are primarily particulate and can be rubbed off the surface readily. Little or no dye, e.g. methylene blue, will adhere to the coated area upon rinsing the dyed slide in water.

In contrast to the film forming silicas, organic film formers, such as polyvinyl alcohol, polyvinyl pyrrolidone, dimethyl hydrantoin formaldehyde, gelatin, etc. have proven unsatisfactory and tend to produce such harmful effects as a significantly lower development rate, pin-pointing, formation of gas bubbles under the topcoating during development, and serious residual developer stain or discoloration.

The glossy silica topcoatings may be prepared by dip, knife, bar, brush or roller coating of the photoconductive copysheet surface with an aqueous sol of the film forming silica, or, if desired, by such techniques as doctoring, gravure offset, etc. to insure uniform coating thickness. Other coating techniques, including those employed in the photographic art, may also be used. Generally, any coating method used for coating a uniform layer of low viscosity material upon a non-absorbent substrate can be utilized. Surfactants, either cationic or non-ionic, may be included in the aqueous silica sol to enhance wetting characteristics and improve the uniformity of the resultant coating. When used, such surfactants are employed at low concentration to avoid fogging the photoconductive coating. Surfactant concentrations are preferably below 0.06% based on silica weight. Wetting characteristics may also be enhanced by including a water-miscible organic solvent, up to about 20% by volume, in the aqueous sol. Lower alkyl alcohols, such as isopropanol and methol, are particularly desirable for this purpose. Generally, the volatility of the water miscible organic solvent should be close to that of water to prevent "orange peel" caused by non-uniform solvent loss during the drying of the silica topcoating.

Coating thickness is important in obtaining the improvements discussed herein. Although the coating weights will vary depending on the degree of gloss desired and consequently on the physical nature of the photoconductive surface, the dry coating weight must be thick enough to provide a continuous glossy topcoating but thin enough to avoid any noticeable excessive "crazing" or minute crack formation in the silica topcoating. Crazing is aggravated by uneven or excessively rapid drying of the wet silica coating, e.g. by elevated temperature drying, as is known in paint technology. Air drying at about room temperature is therefore a preferred embodiment, although other drying procedures can be employed with care to prevent undue crazing.

It has been found that extended aging, particularly at elevated temperatures, can decrease water permeability of the silica film. This problem and the problem of pin-pointing may be minimized by incorporating sulfate ion into the silica film, e.g. by adding various ionizable sulfates, including such inorganic sulfates as zinc sulfate, magnesium sulfate, sulfuric acid, etc. to the aqueous sol in an amount insufficient to adversely affect the gloss characteristics of the dry coating, usually up to about 25% by weight of the silica. Within the silica coating weight range encompassed by the minimum weight to

effect the desired continuous film and gloss characteristics and the maximum rate at which crazing of the film observable by the naked eye is produced, coating weight of the silica on the photoconductive copysheet surface can be adjusted to obtain the desired balance of properties, such as maximum gloss with good water permeability and fast electrolytic development rate. From about 0.1 to about 10, preferably from 1 to 6, grams of silica per square meter has proven satisfactory in most cases. With coating weights above about 10 grams of silica per square meter the electrolytic development rate becomes relatively slow. For lower gloss papers, the lower coating weights are employed.

The transparent cohesive silica films of this invention may also include various other additives, including the developer materials themselves (e.g. zinc, silver and other metal salts, electrolytically reducible dyes), and a wide variety of other materials such as filter dyes, AlOOH, ammonium persulfate, ceric sulfate, HCl, HNO<sub>3</sub>, H<sub>3</sub>PO<sub>4</sub>, ZnCl<sub>2</sub>, ZnF<sub>2</sub>, Zn(NO<sub>3</sub>)<sub>2</sub>, Mg(NO<sub>3</sub>)<sub>2</sub>, acetamide, MgSO<sub>4</sub> urea, acrylamide, quinone, acetic acid, thiourea, N,N'-methylene bis-acrylamide, ethylene diamine tetracetic acid, ascorbic acid, hydroquinone, phenols, morpholine, sucrose, carbowax, etc. Up to about 20 weight percent, preferably below about 10 weight percent, based on the weight of film forming silica, of non-film forming silicas and colloidal boehmite with an average particle size below about 100 millimicrons may also be included in the silica sol formulation. Any additive employed should not impair the transparency and other of the earlier mentioned useful properties of the topcoating. If a paper of lower gloss is desired, one may either apply a thinner coating of the film forming colloidal silica, as noted earlier, or incorporating into the silica sol a non-film forming silica of larger particle size to provide a semi-gloss or matte surface, usually up to about 20 weight percent of the film forming silica.

Although the glossy silica layers of the invention are usually coated directly onto the photoconductive surface, they may also be coated onto intermediate layers or materials which are themselves in contact with the photoconductive surface. Thus, for example, various photoconductive copysheets having a thin, light transmissive indium oxide developer coating on the photoconductive layer, as described in United States patent application Serial Number 848,272, filed October 23, 1959, may be overcoated with the glossy silica layers of this invention. Moreover, various other photoconductive copysheets are provided with a gelatin coating containing the desired developer materials, as exemplified in United States Serial Number 575,070, now U.S. 3,010,883, and these may also be overcoated with the glossy silica layers of this invention. As used herein, therefore, the term "superimposed on" includes both direct and indirect contact with the underlying photoconductive layer.

After the silica coated photoconductive copysheets of this invention are developed, particularly when a silver salt is included in the developer solution, a stabilization step may be desired to prevent discoloration of the background area by entrapped developer in the silica overcoating. Treatment of the copysheet surface with any of the silver stabilizers employed in the photographic art, e.g. quaternary ammonium halides (such as "Triton 400"), saccharine, ethylene thiourea, etc. may be used for this purpose.

Photoconductive copysheet constructions which can be coated with these film forming silicas have been described above with reference to other United States patent applications. Useful highly photoconductive materials include zinc oxide, indium oxide, cadmium sulfide, etc. The photoconductive particulate materials are uniformly dispersed in an insulating binder matrix, e.g. a butadiene-styrene copolymer, etc. and are usually coated onto an electrically conductive backing, e.g. aluminum foil, polyester or other plastic film vapor coated with aluminum

silver, etc. The backing need not necessarily be electrically conductive if such photoconductive copysheets are to be developed by electrostatic techniques. Sensitizing dyes, such as Phosphine R (C.I. 788), Patent Blue (C.I. 672), xylene cyanol (C.I. 715), etc., are usually included in the photoconductive layer to broaden the spectral response of the photoconductor.

The electrolytic image reproduction process, in which the copysheets of this invention may be used, has made possible the direct copying of microfilm reproduction of printed pages of books, papers and the like within a short period of time from initial exposure to the light image to delivery of the completed print. The improved copysheets of this invention are valuable because of their smudge resistance and ability to provide prints or reproductions having significantly higher image density, greater contrast and good definition without significant loss of such other properties as resistance to pinpointing and a relatively rapid development rate. Also, these improved photoconductive copysheets have made photoconductive copysheets suitable for printing continuous tone black and white negatives as well as for making monochrome prints from continuous tone color negatives.

To measure the effect of a film forming silica overcoating on image properties, samples of a photoconductive zinc oxide copysheet (4.6/1 weight ratio of zinc oxide to 30/70 mol ratio copolymer of butadiene/styrene on aluminum foil laminate backing) were overcoated with a 110 line gravure roll using the following film forming silica dispersion:

60 parts by weight film forming silica sol (Nalcoag 1034, 34 wt. percent  $\text{SiO}_2$ )  
33.4 parts by weight water  
6 parts by weight methyl alcohol  
0.6 part by weight  $\text{ZnSO}_4 \cdot 7\text{H}_2\text{O}$

A sample of both the uncoated and the silica overcoated copysheets was then exposed through a 0-3 neutral density continuous wedge to 300 foot candles of incident light. FIGURES 1-3 represent a plot of the diffuse reflection density vs. the log relative exposure for various developers, curves A and B being the uncoated and coated results respectively in each figure.

In FIGURE 1 a ten second exposure was used. Electrolytic development was accomplished by immersing the exposed sheets in a developer containing 0.66 wt. percent silver nitrate, 1.8 wt. percent ethylene thiourea, 1 wt. percent glacial acetic acid, 5 wt. percent magnesium acetate and 91.54 wt. percent distilled water, the sheets being connected as cathode, and electrolyzing for 9 seconds at an applied voltage of 10 volts. The total current on-time was 45% of the total immersion time, since the electrolysis was cycled to reduce polarization effects.

In FIGURE 2 a ten second exposure was also used. Electrolytic development was achieved by immersing the exposed sheets in a developer containing 20 parts by weight  $\text{NiCl}_2 \cdot 6\text{H}_2\text{O}$ , 4 parts ammonium chloride, 4 parts of 28% aqueous ammonium hydroxide, and 200 parts of distilled water (pH of 6.5), the sheets being connected as cathode, and electrolyzing continuously for 5 seconds at a voltage of 25 volts.

In FIGURE 3 a five second exposure was used. Electrolytic development was accomplished by immersing the exposed sheets in a developer containing 2 wt. percent silver nitrate, 2 wt. percent magnesium nitrate and 96% distilled water, the sheets being connected as cathode, and electrolyzing for 0.5 second at 60 volts. The total current on-time was 10% of the total immersion time, since the electrolysis was cycled to reduce polarization effects.

From the curves of FIGURES 1-3, the higher maximum density, steeper gradient and lower fog are evident, as compared to the uncoated copysheets. Moreover, another significant property of the silica overcoated copysheets is their ability to improve both density and contrast with continued extended development, as contrasted

with the uncoated copysheets which tend to reach a maximum diffuse reflection density of about 0.9 or less.

Photoconductive zinc oxide copysheets (4.6/1 weight ratio  $\text{ZnO}$  to Pliolite S-7 binder on aluminum laminate backing) were developed with an aqueous solution containing silver salt and thiourea after an extended exposure to light (i.e. saturation exposure). By controlling development time, varying image densities were obtained up to the maximum value of about 0.9 diffuse reflection density, as shown in FIGURE 4, curve A. By overcoating these developed copysheets with a film forming silica sol (Nalcoag 1050, deionized, 3-4 grams per square meter dry coating weight) the optical densities, as measured by the diffuse reflection densities, were increased up to about 0.2 unit, as shown in FIGURE 4, curve C. This may be attributed to the optical effect resulting from less light being reflected from a glossy surface and hence greater light penetration and absorption. Other photoconductive zinc oxide copysheets were overcoated with the same silica sol at the same coating weight level before exposure and development. After exposure and development in the same manner, the optical density values were markedly higher, as shown in FIGURE 4, curve B. These results indicate that higher diffuse reflection density values cannot be attributed solely to optical effect, although the actual mechanism is not fully known.

To a deionized aqueous sol of film forming silica containing 28.5 parts by weight of silica in 66.5 parts of water (i.e. Nalcoag 1034A) was added 4.75 parts of isopropanol and 0.25 part of concentrated sulfuric acid. This sol was then coated onto a photoconductive copysheet (zinc oxide in a binder matrix of butadiene-styrene copolymer on a backing of a polyethylene terephthalate vapor coated with aluminum) in a dry coating weight of 3 to 4 grams per square meter. A highly glossy finish was produced which was not removed with pressure-sensitive cellophane tape in the standard test. This overcoated copysheet was exposed and developed with an aqueous silver developer (2%  $\text{AgNO}_3$  and 2% magnesium nitrate) to produce a dense, stable, high contrast image with excellent definition and good resistance to smudging and without pinpointing. Similar results were obtained with the use of methyl alcohol rather than isopropanol and zinc sulfate rather than sulfuric acid.

As mentioned earlier, the film forming silica layer must be water permeable. A simple test for water permeability may be conducted by coating a magnesium plate with the silica sol to be evaluated and drying the coating either with a hot air current or at ambient room conditions to form a continuous coating on the plate. A few drops of dilute aqueous hydrochloric acid solution is then placed on the coated surface. After a few minutes the coating is physically removed and any etching of the metallic zinc substrate is noted. Water permeability is indicated by such etching.

Various other embodiments and modifications will be apparent to those skilled in the art from the foregoing disclosure without departing from the spirit and scope of this invention.

I claim:

1. In a photoconductive copysheet capable of electrolytic development the improvement which comprises, superimposed on the photoconductive surface thereof, a continuous, glossy, transparent, cohesive and water permeable layer comprising a film forming silica having an average particle size range from about 1 to about 100 millimicrons and a sulfate, said layer having a silica coating weight of from about 0.1 to about 10 grams per square meter and a sulfate content up to about 25 percent by weight of said silica, said layer being essentially free of alkali metal ions.

2. In a photoconductive copysheet capable of electrolytic development the improvement which comprises, superimposed on the photoconductive surface thereof, a continuous, glossy, transparent cohesive and water per-

meable layer comprising a film forming silica having an average particle size range from about 1 to about 100 millimicrons and a sulfate, said layer having a silica coating weight of about 1 to about 6 per square meter and a sulfate content up to about 25 percent by weight of said silica, said layer being essentially free of alkali metal ions.

3. A process for the preparation of improved photoconductive copysheets capable of electrolytic development which comprises applying over the photoconductive coating thereof a film forming silica sol having an average silica particle size of from about 1 to about 100 millimicrons, said silica sol being essentially free of alkali metal ions, in an amount sufficient to provide a glossy dry coating having essentially no crazing observable by the naked eye and having a coating weight of from about 0.1 to about 10 grams per square meter, and drying said coating to produce a continuous, glossy, transparent, cohesive and water permeable layer superimposed on said photoconductive coating.

4. The process of claim 3 in which said silica sol is an aqueous sol containing up to about 25 weight percent of a sulfate, based on the weight of said silica.

5. The process of claim 3 in which said silica sol is an aqueous sol containing up to about 20 percent by volume of a water miscible organic solvent.

6. The process of claim 3 in which said silica sol is an aqueous sol containing up to about 20 percent by volume of a water miscible lower alkyl alcohol.

7. A photoconductive copysheet capable of electrolytic development which comprises a continuous electrically

10  
5 conductive layer having thereon a thin, continuous and contiguous layer of photoconductive particles in a water-insoluble insulative binder and, superimposed thereon, a thin, continuous, glossy, adherent, transparent, cohesive, water permeable and water insoluble layer comprising a film forming silica, said layer being essentially free of alkali metal ions.

8. A photoconductive copysheet capable of electrolytic development which comprises a continuous electrically conductive layer having thereon a thin, continuous and contiguous layer of photoconductive particles in a water-insoluble insulative binder and, superimposed thereon, a thin, continuous, glossy, adherent, transparent, cohesive, water permeable and water insoluble layer comprising a film forming silica in a coating weight of from about 0.1 to about 10 grams per square meter, said layer being essentially free of alkali metal ions.

9. The copysheet of claim 8 in which the coating weight of said film forming silica is from about 1 to about 6 grams per square meter.

15  
15 10. The copysheet of claim 8 in which said film forming silica layer is essentially free of crazing observable by the naked eye.

25  
25 References Cited in the file of this patent

UNITED STATES PATENTS

|           |                  |               |
|-----------|------------------|---------------|
| 2,244,325 | Bird             | June 3, 1941  |
| 2,886,434 | Owens            | May 12, 1959  |
| 2,901,349 | Schaffert et al. | Aug. 25, 1959 |